

NORMAN MARSHALL, OF WEST NEWTON, MASSACHUSETTS.

ELECTRIC INSULATOR.

1,217,873

1,217,873.

No Drawing.

Specification of Letters Patent. Application filed June 20, 1916. Serial No. 104,783.

Patented Feb. 27, 1917.

173-368

*To all whom it may concern:*

Be it known that I, NORMAN MARSHALL, a citizen of the United States, residing at West Newton, in the county of Middlesex 5 and State of Massachusetts, have invented certain new and useful Improvements in Electric Insulators; and I do hereby declare the following to be a full, clear, and exact description of the invention, such as 10 will enable others skilled in the art to which it appertains to make and use the same.

This invention relates to electric insulators, and more particularly to insulators for lining metal sockets for nitrogen and other 15 incandescent lamps.

Various types of metal lamp sockets used for electric light globes having carbon or tungsten filaments in a vacuum, have a paper or vulcanized fiber insulating lining. 20 A nitrogen lamp, and large sizes of carbon and tungsten filament lamps, should not be used with such a socket, because the heat generated by the lamp when lighted often becomes great enough to burn or char such 25 lining, so as to cause short circuits in the lighting circuit and many times setting fire to the adjoining structure. For this reason metal lamp sockets for use with nitrogen and other large lamps have been condemned by 30 municipal building inspectors and fire insurance companies.

The primary object of the present invention is to provide an electric insulator which has adequate heat resisting properties to 35 permit its use in metal lamp sockets for nitrogen and other high temperature lamps without the danger of failure under high temperature.

Another object of the invention is to provide 40 a process of making insulators by which they may be prepared for the various electrical and heat insulating purposes.

With these objects in view the invention consists in the improved insulator and the 45 process of making the same, which are hereinafter described and particularly defined in the claims.

In the preferred process of making insulating tubes or linings for lamp sockets, 50 blanks of a predetermined shape are cut from sheet asbestos and saturated with an emulsion of sodium silicate and linseed oil. The saturated sheet is then rolled with considerable pressure upon an arbor or mandrel 55 and carefully removed and permitted to dry in the air until it hardens and can be

handled. The dried tube is then dipped in linseed oil and permitted to cure or oxidize in the air from one to four days, depending upon the size and thickness of the tube, and 60 then placed in a drying oven heated by steam for a shorter time. The coated and dried tube is then baked in an oven at a temperature of from 450° to 550° F. until the tube ceases to give off volatile material 65 or smoke, this generally taking from 5 to 60 minutes according to the thickness and the size of the tubes. In making linings for the well-known type of lamp socket which has a reduced diameter for a portion of its 70 length, the tube, which has been formed on the mandrel, is coated with linseed oil to make it more flexible, and allowed to dry. When dry, the tube is drawn in dies to form a lining similar in shape to that shown and 75 described in my Patent No. 784,695 dated March 14, 1905. The drawn tube is then baked in an oven at a temperature from 425° to 700° F. until volatilization ceases.

The product thus obtained is a rigid tube 80 or lining having a brown or black color and possessing excellent heat and electric insulating properties.

The emulsion of sodium silicate and linseed oil is preferably made by mixing one 85 part of sodium silicate with one part of raw linseed oil. These proportions, however, are not essential, since good results have been obtained with a mixture containing two parts of sodium silicate to one part of linseed oil, and with a mixture containing two parts of linseed oil to one part of sodium silicate. This emulsion undoubtedly contains a certain amount of sodium soaps, due 90 to the unstable character of the sodium silicate and the presence of free alkali in the sodium silicate. In place of the sodium silicate any of the soluble silicates such as potassium or the double salt of sodium and potassium, may be employed. While linseed oil seems to have the better drying 95 properties, other oxidizable oils, such as soybean oil and tung-oil, may be employed in the place of the linseed oil.

The finished product is characterized by 105 the following chemical and physical properties: When the asbestos treated with the above emulsions is dried in the air, the sodium silicate becomes partially dehydrated and the linseed oil oxidizes. In baking the dried product in an oven at a temperature above 400° F., the sodium silicate is dehy- 110

drated and the oil is polymerized or resini-  
fied. While the chemical constitution of the  
baked product is not known, it undoubtedly  
contains some reaction products such as the  
5 sodium salts of acetic and palmitic acids, but  
since these are covered with the polymerized  
oil they do not take up moisture or destroy  
the dielectric properties of the insulator.  
The dehydrated sodium silicate is dis-  
10 tributed throughout the compound and has  
its well-known fireproofing properties to  
resist the action of heat in breaking down  
the structure of the tube. The solid resini-  
fied oil has excellent dielectric properties,  
15 and since it is formed at a very high temper-  
ature, it is a good heat insulator. The as-  
bestos is a good electric insulator and is  
very resistant to heat. The solidified lin-  
seed oil as well as the sodium silicate act  
20 as binders in building up and maintaining  
the structure of the tube and preventing the  
structure of the asbestos from breaking  
down under heat. The coating of linseed  
oil which is placed upon the tube after the  
25 emulsion has dried thereon, becomes oxi-  
dized and polymerized in the baking opera-  
tion and gives the finished product a var-  
nished appearance.

The curing operation of the tube is pref-  
30 erably conducted for a long period at mod-  
erate temperatures in the air, so that the oil  
may become well oxidized. However, the  
curing operation may be accelerated by dry-  
ing in a steam heated oven in the presence  
35 of air, or by drying a shorter time in the  
air and finishing the drying in the steam  
heated oven.

Although it is preferred to bake the prod-  
uct between 425° and 500° F., an excellent  
40 product may be obtained by temperatures up  
to 750° F. The greater the degree of tem-  
perature used in baking, the darker the tube  
becomes, until it turns black. A tube baked  
at the higher degrees of temperature is very  
45 stiff and brittle, and although it has a  
greater strength than the tube made at the  
lower temperature, the flexibility of the tube  
having the brown color is very advantageous  
for use in insulating metal lamp sockets.

50 While asbestos is preferably used as a car-  
rier, an insulating tube of good quality may  
be made with a carrier consisting of a cot-  
ton fiber paper or a flax paper. The heat  
resisting and insulating properties of the  
55 hardened linseed oil and dehydrated silicate  
will protect this type of paper so that it may  
be safely used for the smaller sizes of nitro-  
gen lamps.

Sodium silicate has well-known fire pro-  
60 tecting properties, and if it is desired to in-  
crease the heat resisting properties of the  
composition, the percentage of sodium sili-  
cate is increased. The amount of silicate,  
however, is limited, since it makes the tube  
65 brittle. By mixing the linseed oil with the

silicate, however, the finished product can  
be controlled to get practically any desired  
heat resisting property and still have the  
proper strength and flexibility to suit the va-  
rious purposes for which the insulator is to 70  
be used.

While the electric insulator has been de-  
scribed as being especially adapted for insu-  
lating metallic lamp sockets, it is not limited  
to such use but may be used for practically 75  
any heat or electric insulating purpose.

The preferred form of the invention hav-  
ing been thus described, what is claimed as  
new is:—

1. An insulator comprising a dielectric 80  
carrier impregnated with a dehydrated soluble  
silicate and a polymerized oil.

2. An insulator comprising a dielectric  
heat resisting carrier impregnated with a de-  
hydrated soluble silicate and an oxidized 85  
vegetable oil.

3. An insulator comprising asbestos im-  
pregnated with a dehydrated soluble silicate  
and a polymerized and oxidized vegetable  
oil. 90

4. An insulating lining for lamp sockets  
comprising a tube of sheet asbestos which is  
impregnated with decomposition and reaction  
products of an emulsion of sodium silicate  
and raw linseed oil, which has been oxidized 95  
and baked at a comparatively high tempera-  
ture, and characterized by its heat resisting  
and dielectric properties.

5. An insulating lining comprising an as-  
bestos tube which is impregnated with de-  
composition and reaction products of a mix-  
ture of from 30% to 70% linseed oil with  
from 70% to 30% of a soluble silicate which  
has been oxidized and baked at a high tem-  
perature, and characterized by its heat re-  
sisting and dielectric properties, said insula-  
tor varying in color from brown to black  
in accordance with the higher degree of tem-  
perature employed in baking, the black ma-  
terial being more brittle than the brown. 100  
105  
110

6. An insulator comprising a shaped heat  
resisting carrier impregnated with a dehy-  
drated soluble silicate and polymerized  
vegetable oil, and coated with an oxidized  
and resined vegetable oil. 115

7. An insulating lining consisting of an  
asbestos tube having its diameter reduced  
for a portion of its length, said tube being  
impregnated with sodium silicate and poly-  
merized linseed oil, and characterized by its 120  
brown-black color and rigid structure.

8. The process of making an insulator  
comprising saturating a heat resisting car-  
rier with a soluble silicate and an oxidizable  
oil, oxidizing and baking the impregnated 125  
carrier.

9. The process of making an insulator  
comprising saturating a sheet of a heat re-  
sisting carrier with an emulsion of a soluble  
silicate and oxidizable vegetable oil, shaping 130

the saturated sheet and drying it in an oxidizing atmosphere, and baking the oxidized article at a comparatively high temperature.

10. The process of making an insulator comprising saturating a sheet of asbestos with an emulsion of sodium silicate and linseed oil, shaping the saturated sheet into a lining tube and drying it in the air, and then baking the dried tube to solidify the silicate

10 and oil.

11. The process of making an insulator comprising saturating a sheet of asbestos with an emulsion of a soluble silicate and an oxidizable vegetable oil, shaping the saturated sheet and drying it in an oxidizing atmosphere, coating the dried article with an oxidizable oil and curing it in an oxidizable atmosphere, and then baking the coated article at a comparatively high temperature.

12. The process of making an insulator 20 comprising saturating sheet asbestos in a mixture of from 30% to 70% of sodium silicate with from 70% to 30% linseed oil, shaping the saturated sheet and drying it in the air, coating the shaped article with the linseed oil, drying the coated article in the air, and baking the dry-coated article at a temperature of from 400° to 650° F. 25

13. The process of making a lining for lamp sockets comprising saturating sheet asbestos with an emulsion of sodium silicate and linseed oil, forming a tube of the saturated sheet, drying the tube, drawing the tube to reduce the diameter of a portion of its length, and then baking the drawn tube 35 in an oven.

NORMAN MARSHALL.